# EUROPEAN PATENT APPLICATION

(11) **EP 1 992 721 A1**
(43) Date of publication of application: **19.11.2008**
(21) Application number: 07076056.6
(22) Date of filing: 07.12.2007
(51) Int. Cl.: D01D 5/00

(54) **Fibrous structures, processes and devices for preparing the same**

(30) Priority: 18.05.2007 EP 07009995
(71) Applicant: Universiteit Gent, 9000 Gent (BE)
(72) Inventor: Westbroek, Philippe, 9200 Dendermonde (BE); Van Camp, Tamara, 9000 Gent (BE); Gasana, Emmanuel, 9000 Gent (BE); De Dieu Hakuzimana, Jean, 9790 Wortegem-Petegem (BE); De Vrieze, Sander Aimée Pierre, 9700 Oudenaarde (BE)
(74) Representative: Bird, William Edward

(57) **Abstract**

An electrospinning device is described for producing fibrous porous structures. The device is adapted for providing a predetermined distance profile for the distance between the outlets and the receiving surface along the direction of lengthwise growth of the fibrous structure. A fibrous structure obtained by the described electrospinning device is also described which comprises fibers, wherein the diameter of the fibers has a predetermined profile along a dimension of the electrospun fibrous structure.

## Description

### Technical field of the invention

The present invention relates to a fibrous structure, a process and a device for manufacturing the same. In particular, the present invention relates to methods and systems for electrospinning of fibrous structures and resulting products such as e.g. nanofibrous structures and their use.

### Background of the invention

Nanofibrous structures are useful in a variety of applications in the fields of clothing, filtering, medicine and defense. There is a strong interest in nanofibrous structures based on their high porosity for absorption, immobilization and inclusion of chemicals, solvent, solutions, melts and liquid phases. In many applications where high absorption is preferred, an absorption capacity of about 5 mL.cm⁻² is preferably obtained. In the same applications large nanofibrous structures are preferred. In order to guarantee homogeneous absorption behaviour over the structure it is useful to obtain a regular thickness over the entire structure. In addition, application of nanofibrous structures in filtration requires a strong structure with high dirt holding capacity, multilevel filtration, low cut-off value and limited pressure drop.Nanofibrous structures can be produced using an electrospinning setup. A basic setup is shown in FIG. 1 and consists of a high voltage source 1, an anesthesia pump 2, the pump comprising a syringe 3 that contains a polymer solution 4 and the pump transporting polymer solution towards the tip of a metallic needle 5, said needle positioned in a spinneret 6, said spinneret comprising an upper 7 and a lower 8 conductive plate. An electrical field is applied over the upper and lower plate resulting in an extrusion ability of the polymer solution at the tip of the needle towards the surface of the lower element. The electrical field created, causes the polymer solution to overcome the cohesive forces that hold the polymer solution together. As a result of cohesive force compensation by the electrical field a jet will be drawn from the polymer solution droplet, which forms nano-dimensioned fibres, finally collected at the lower plate. Typical dimensions of the deposited structures are circular surfaces with a diameter of about 10 to 15 cm. Therefore, with a single nozzle system, it is not possible to obtain the large surface areas required for many applications in an economic feasible way.

In US2002/0175449 an apparatus and method for electrospinning polymeric fibers and membranes is disclosed. The method involves controlling the electrical field strength at the spinneret tip by adjusting the electric charge on a field modifying electrode to provide a fiber of controlled diameter. By changing the electrostatic potential, the jet stream acceleration is altered, resulting in varying the diameter of the formed nano-fiber. This electrostatic potential variation changes the jet stream stability, and therefore, corresponding changes in the composite electrode can be used to stabilize the new jet stream. The distance between two neighbouring spinnerets may- be-varied to optimize the electrical field, i.e. such that the electric fields for the individual spinnerets do not influence each other.

### Summary of the invention

It is an object of the present invention to provide innovative devices or methods for producing fibrous (e.g. nanofibrous) structures. It is an advantage of embodiments according to the present invention that fibrous structures comprising fibres, wherein the diameter of the fibres varies, e.g. decreases, along a dimension of the electrospun fibrous structure can be obtained and methods and apparatus for producing them. It is furthermore an advantage of embodiments according to the present invention that fibrous structures with good liquid uptake are provided and methods for producing them. It is also an advantage of embodiments according to the present invention that fibrous structures with good control release and filtration properties are provided and methods for producing them. It is an advantage of embodiments according to the present invention that fibrous structures can be provided in an economic viable way. It is an advantage of embodiments according to the present invention that fibrous structures with a combination of two or more of the above described advantages can be obtained. It is an advantage of embodiments according to the present invention that laminated structures can be made. It is an advantage of embodiments according to the present invention that a good overlap is obtained using movement of the different nozzles with respect to the collector.

The above objective is accomplished by a method and device according to the present invention.

The invention relates to an electrospinning device for producing fibrous structures, said electrospinning device comprising a set of outlets for outputting solution or melt, a receiving surface for receiving output from said set of outlets, wherein said receiving surface is adapted to move in a first direction parallel to said receiving surface, said movement being responsible for the lengthwise production of said fibrous structure, a voltage source for generating a potential difference between said set of outlets and said receiving surface, characterized in that said electrospinning device is adapted for providing a predetermined distance profile for the distance between the outlets and the receiving surface along said first direction. The predetermined distance profile may be an increasing distance profile or a decreasing distance profile. The predetermined distance profile may be a monotonously increasing distance profile or a monotonously decreasing distance profile. It is an advantage of embodiments according to the present invention that devices are provided allowing to produce fibrous structures comprising fibres, wherein the diameter of said fibres decreases along a dimension of said electrospun fibrous structure and wherein the variance of the fibres diameter in any section perpendicular to said dimension, is below a predetermined level, e.g. below 10%. In embodiments of the present invention, the diameter of said fibres decreases monotonously along a dimension of said electrospun fibrous structure. In other embodiments of the present invention, the diameter of the fibres is according to a predetermined fibre diameter profile along a dimension of the electrospun fibrous structure. For example, the diameter of said fibres decreases monotonously and continuously along a dimension of said electrospun fibrous structure.

In embodiments of the present invention, the set of outlets comprises subsets of outlets and each of said subset of outlets consists of outlets equidistant to said receiving surface and the distance between each subset and the receiving surface varies according to a predetermined distance profile along the direction of lengthwise growth of the fibrous structure. It is an advantage of embodiments of the present invention that layered structures comprising two or more adjacent layers can be produced, wherein each layer having two neighboring layers is composed of fibers having an average diameter smaller than the average diameter of the fibers of one of its neighboring layer and larger than the average diameter of the fibers of its other neighboring layer.

In embodiments of the present invention, the set of outlets may be comprised in a plane inclined at an angle relatively to the receiving surface. This is advantageous as it permits the production of fibrous structure comprising fibers wherein the diameter of said fibers continuously decreases along a dimension of the fibrous structure.

According to embodiments of the present invention, the distance of the nozzles to the collector can be varied during the electrospinning process as well as before and/or after the process.

In embodiments of the present invention, at least two neighbouring outlets of said set of outlets may be separated from one another by a distance of at least 1 cm. It is an advantage of embodiments according to the present invention that devices are provided allowing to produce fibrous structures with high porosity. At least two neighbouring outlets of said set of outlets may be separated by a distance of at least 2 cm. It is particularly advantageous to separate two neighbouring outlets by a distance of at least 4 cm and very advantageous to separate two neighbouring outlets by a distance of at least 8 cm. Each two outlets of said set of outlets may be separated from one another by a distance of at least 1 cm, advantageously a distance of at least 2 cm, more advantageously of at least 4 cm and very advantageous to separate two neighbouring outlets by a distance of at least 8 cm.. In other words, there is at least one outlet (e.g. a nozzle) for which the distance to the closest other outlet is at least 1 cm, advantageously at least 2 cm, more advantageously at least 4 cm and very advantageous to separate two neighbouring outlets by a distance of at least 8 cm.. A majority or all of said outlets may be separated from the other outlets by a distance of at least 1 cm, advantageously at least 2 cm, more advantageously at least 4 cm and very advantageous to separate two neighbouring outlets by a distance of at least 8 cm.. It is an advantage of embodiments according to the present invention that devices are provided allowing production of fibrous structures that are strong, have high porosity and straight fibres. As an optional feature, the outlets (e.g. needles) are positioned in a triangle setup or a multiple thereof.

In embodiments of the present invention, the distance between the outlets may be adapted for obtaining a fibrous structure comprising at least 50% of fibers substantially free of cross-links to neighboring fibers. It is an advantage of embodiments according to the present invention that devices are provided allowing production of fibrous structures wherein only a low degree of cross-linked fibers is present.

In embodiments of the present invention, the distance between the outlets may be adapted for obtaining a fibrous structure comprising at least 50% of straight fibers.

In embodiments of the present invention, the device may be adapted for applying one or more relative movements between said set of outlets and said receiving surface, e.g. at any stage of the processing.

In embodiments of the present invention, the set of outlets may be adapted to be movable reciprocally in a direction parallel to said receiving surface and perpendicular to said first direction. This is advantageous because it permits the outputted umbrellas of solution or melts to overlap on the receiving surface.

The device may comprise control means for varying the diameter of the produced fibres.

In embodiments of the present invention, the means for varying the diameter of the produced fibres may be control means for altering the distance between said first plane and said receiving surface during or outside the production of the fibrous structure. As an optional feature, the lower and the upper section are adapted to be moveable perpendicularly to each other.

In embodiments of the present invention, the device may be adapted for generating a plurality of fibers, whereby at least 50% of said plurality of fibers may comprise an average diameter between 3 and 2000 nm.

In embodiments of the present invention, the device may be adapted for using a polymer solution or melt comprising at least one of a polyamide, polystyrene, polycaprolactone, polyacrylonitrile, polyethylene oxide, polylactic acid, polyacrylic acid, polyesteramide, polyvinyl alcohol, polyimide, polyurethane, polyvinylpyrrolidon, collagen, cellulose, chitosan, methacrylates, silk or metal.

In embodiments of the present invention, the device may further comprise a recipient for containing a solution or melt to be electrospun from said outlets, and means for providing said solution or melt to said outlets.

As an optional feature, said recipient may contain a polymer solution or melt.

As an optional feature, the device may allow the production of nanofibrous structures with a width between 15 cm and 10.000 cm.

As another optional feature, the device may comprise a surrounding element over the spinneret to avoid instability and to allow solvent removal and recuperation.

As another optional feature, the device may comprise a temperature control system that allows to control the temperature in the range of 280 - 1500 K.

The present invention also relates to a method for producing fibrous structures, said method comprising the steps of providing a set of outlets for outputting solution or melt, providing a receiving surface for receiving output from said set of outlets, moving said receiving surface in a first direction parallel to said receiving surface, applying a potential difference between said set of outlets and said receiving surface, and, during said moving and applying, providing a solution or melt to said outlets, wherein the distance between the outlets and the receiving varies along a predetermined distance profile along the direction of lengthwise growth of the fibrous structure. The predetermined distance profile may be an increasing or decreasing distance profile, e.g. a monotonous increasing or monotonous decreasing distance profile. At least two neighbouring outlets of said two or more outlets may be separated by a distance of at least 1 cm, advantageously at least 2 cm, more advantageously at least 4 cm and very advantageous to separate two neighbouring outlets by a distance of at least 8 cm. Each two of said set of outlets may be separated from one another by a distance of at least 1 cm, advantageously at least 2 cm, more advantageously at least 4 cm and very advantageous to separate two neighbouring outlets by a distance of at least 8 cm.

The variation of the distance between the outlets and the receiving surface may optionally be obtained by adapting the distance between said neighbouring outlets and said receiving surface during the production of the fibrous structure.

The distance may be adapted by providing a relative movement between said set of outlets and said receiving surface.

As an advantageous optional feature, the method may further comprise the step of moving reciprocally at least one of said set of outlets and/or said receiving surface in a direction parallel to said receiving surface and perpendicular to said first direction.

The method may be adapted for generating a plurality of fibers, whereby at least 50% of said plurality of fibers comprises an average diameter between 3 and 2000 nm.

The method may be adapted for using a polymer solution or melt comprising at least one of a polyamide, polystyrene, polycaprolactone, polyacrylonitrile, polyethylene oxide, polylactic acid, polyacrylic acid, polyesteramide, polyvinyl alcohol, polyimide, polyurethane, polyvinylpyrrolidon, collagen, cellulose, chitosan, methacrylates, silk or metal.

As an optional feature, a voltage difference of between 100 V and 200000 V may be applied over the set of outlets and the receiving surface.

As another optional feature, the pump rate of the polymer solution or melt per outlet may be between 0.01 and 500 mL h⁻¹.

As an optional feature, the solutions or melts may contain an additional compound, such as compounds with antibacterial, pharmaceutical, hydrophobic/hydrophilic, anti corrosion, catalytic, oxidative/reductive and other properties.

The present invention also relates to an electrospun fibrous structure manufactured using a method according to embodiments of the present invention as described above.

The present invention also relates to an electrospun fibrous structure comprising fibres, wherein the diameter of said fibres varies according to a predetermined fibre diameter profile along a dimension of said electrospun fibrous structure and wherein the variance of the fibres diameter in any section perpendicular to said dimension, is below 10%.

In embodiments of the present invention, the structure comprises at least 50% of straight fibers, wherein at least 50% of straight fibers consists of 50% or more fibres having segments substantially straight over a distance of 5 µm.

The electrospun fibrous structure may comprise at least 50% of fibers that is substantially cross-link free with respect to neighbouring fibers.

The electrospun fibrous structure may comprise at least 50% of randomly oriented fibers.

The electrospun fibrous structure may have a porosity of at least 65%.

50% or more of its fibers may have an average diameter between 3 and 2000 nm, preferably equal or above 10 nm, preferably equal or below 700 nm.

The present invention also relates to an electrospun fibrous structure comprising two or more layers, wherein each of said layers is composed of fibers having an average diameter different from the average diameter of the fibers of an adjacent layer.

In embodiments of the present invention, the fibrous structure comprises two or more adjacent layers, wherein each layer having two neighbouring layers is composed of fibers having an average diameter of a predetermined size which may be larger or smaller than the average diameter of the fibers of its neighbouring layer. In some embodiments the average diameter of the fibers may be smaller than the average diameter of the fibers of one of its neighbouring layer and larger than the average diameter of the fibers of its other neighbouring layer. The diameter may for example decrease as function of the depth, increase as function of the depth, first decrease and then increase as function of the depth, first increase and then decrease as function of the depth, etc.

Particular and preferred aspects of the invention are set out in the accompanying independent and dependent claims. Features from the dependent claims may be combined with features of the independent claims and with features of other dependent claims as appropriate and not merely as explicitly set out in the claims.

Although there has been constant improvement, change and evolution of devices in this field, the present concepts are believed to represent substantial new and novel improvements, including departures from prior practices, resulting in the provision of more efficient, stable and reliable devices of this nature.

The teachings of the present invention permit the design of improved methods and apparatus for manufacturing fibrous structures with enhanced properties.

The above and other characteristics, features and advantages of the present invention will become apparent from the following detailed description, taken in conjunction with the accompanying drawings, which illustrate, by way of example, the principles of the invention. This description is given for the sake of example only, without limiting the scope of the invention. The reference figures quoted below refer to the attached drawings.

### Brief description of the drawings

FIG. 1 is a schematic representation of a side view of an electrospinning setup according to the prior art.
FIG. 2 is a schematic representation of a perspective view of an electrospinning device according to an embodiment of the present invention.
FIG. 3 is a schematic representation of a perspective view of an electrospinning device according to another embodiment of the present invention.
FIG.4 is a schematic representation of a perspective view of an electrospinning device according to another embodiment of the present invention.
FIG. 5 is a schematic representation of a planar view of the positioning of the outlets for use in an electrospining device according to embodiments of the present invention.
FIG. 6 is a schematic representation of a planar view of the positioning of the outlets for use in an electrospining device according to other embodiments of the present invention.
FIG. 7 shows an example of a laminated nanofibrous structures obtainable using methods and systems according to embodiments of the present invention.
FIG. 8 shows an example nanofibrous structure having a layered structure comprising one layer with an average diameter of 500nm, as can be obtained using a method according to an embodiment of the present invention.
FIG. 9 illustrates another layer of the example nanofibrous structure of FIG. 8 having an average diameter of 300nm.
FIG. 10 shows the relationship between the nanofibre diameter and the distance between outlets and the receiving surface for the example of FIG. 8, as can be used in an embodiment of the present invention.
FIG. 11 illustrates an example nanofibrous structure having a layered structure comprising at one side fibres with an average diameter of 285nm, as can be obtained using a method according to an embodiment of the present invention.
FIG. 12 illustrates the other side of the example nanofibrous structure of FIG. 8 having an average diameter of 180nm.
FIG. 13 shows a profile of the distance between outlets and the receiving surface on the one hand and the average nanofibre diameter for different concentrations, as can be used according to an embodiment of the present invention.

### Description of illustrative embodiments

The present invention will be described with respect to particular embodiments and with reference to certain drawings but the invention is not limited thereto but only by the claims. The drawings described are only schematic and are non-limiting. In the drawings, the size of some of the elements may be exaggerated and not drawn on scale for illustrative purposes. The dimensions and the relative dimensions do not correspond to actual reductions to practice of the invention.

Furthermore, the terms first, second, third and the like in the description and in the claims, are used for distinguishing between similar elements and not necessarily for describing a sequence, either temporally, spatially, in ranking or in any other manner. It is to be understood that the terms so used are interchangeable under appropriate circumstances and that the embodiments of the invention described herein are capable of operation in other sequences than described or illustrated herein.

It is to be noticed that the term "comprising", used in the claims, should not be interpreted as being restricted to the means listed thereafter; it does not exclude other elements or steps. It is thus to be interpreted as specifying the presence of the stated features, integers, steps or components as referred to, but does not preclude the presence or addition of one or more other features, integers, steps or components, or groups thereof. Thus, the scope of the expression "a device comprising means A and B" should not be limited to devices consisting only of components A and B. It means that with respect to the present invention, the only relevant components of the device are A and B.

Reference throughout this specification to "one embodiment" or "an embodiment" means that a particular feature, structure or characteristic described in connection with the embodiment is included in at least one embodiment of the present invention. Thus, appearances, of the phrases "in one embodiment" or "in an embodiment" in various places throughout this specification are not necessarily all referring to the same embodiment, but may. Furthermore, the particular features, structures or characteristics may be combined in any suitable manner, as would be apparent to one of ordinary skill in the art from this disclosure, in one or more embodiments.

Similarly it should be appreciated that in the description of exemplary embodiments of the invention, various features of the invention are sometimes grouped together in a single embodiment, figure, or description thereof for the purpose of streamlining the disclosure and aiding in the understanding of one or more of the various inventive aspects. This method of disclosure, however, is not to be interpreted as reflecting an intention that the claimed invention requires more features than are expressly recited in each claim. Rather, as the following claims reflect, inventive aspects lie in less than all features of a single foregoing disclosed embodiment. Thus, the claims following the detailed description are hereby expressly incorporated into this detailed description, with each claim standing on its own as a separate embodiment of this invention.

Furthermore, while some embodiments described herein include some but not other features included in other embodiments, combinations of features of different embodiments are meant to be within the scope of the invention, and form different embodiments, as would be understood by those in the art. For example, in the following claims, any of the claimed embodiments can be used in any combination.

In the description provided herein, numerous specific details are set forth. However, it is understood that embodiments of the invention may be practised without these specific details. In other instances, well-known methods, structures and techniques have not been shown in detail in order not to obscure an understanding of this description.

The following terms are provided solely to aid in the understanding of the invention.

Unless provided otherwise, the terms "increasing" when applied to a parameter shall be understood as describing an evolution of this parameter toward higher values, said evolution optionally comprising plateaux wherein said parameter has a constant value.

Unless provided otherwise, the terms "decreasing" when applied to a parameter shall be understood as describing an evolution of this parameter toward lower values, said evolution optionally comprising plateaux wherein said parameter has a constant value.

Unless provided otherwise, the terms "continuously or monotonously increasing" when applied to a parameter shall be understood as describing an evolution of this parameter toward higher values, said evolution not comprising plateaux wherein said parameter has a constant value.

Unless provided otherwise, the terms "continuously or monotonously decreasing" when applied to a parameter shall be understood as describing an evolution of this parameter toward lower values, said evolution not comprising plateaux wherein said parameter has a constant value.

The invention will now be described by a detailed description of several embodiments of the invention. It is clear that other embodiments of the invention can be configured according to the knowledge of persons skilled in the art without departing from the technical teaching of the invention, the invention being limited only by the terms of the appended claims.

In a first aspect, the present invention relates to an electrospinning device for producing fibrous structures such as e.g. nanofibrous structures. In an embodiment of the first aspect, the electrospinning device comprises a set of outlets for outputting solution or melt. The electrospinning device of the present invention is a multinozzle device, i.e. a device comprising two or more outlets for outputting solution or melt. The outlets may be of any nature known by the person skilled in the art to be suitable for electrospinning. The outlets are adapted for outputting material, e.g. solution or melt material to be used for the production of the fibers. For instance, the outlets may be nozzles, needles such as e.g. metalic needles, small holes or the likes. In embodiments of the present invention, the two or more outlets are separated from one another by a distance of at least 1 cm. For instance, the outlets may be separated by a distance of 1 to 100 cm. By separating the outlets by 1 or more cm, the fibrous structures obtained are usually stronger, more porous and comprise straighter fibres than for smaller spacing. The relatively large distance between the outlets (e.g. needles) allows a good evaporation of the solvent, thus resulting in high porosity of the fibrous structure obtained. Without being bound by theory this effect may result from a more complete fibre formation process at the moment of collection of those fibers. Advantageously, the distance between the two or more outlets is at least 2 cm, more advantageously 4 cm or more, most advantageously 8 cm or more. The maximum spacing is arbitrary and will for instance depend on the porosity one wishes to achieve.

For a spacing of 1 cm or above between the outlets, the fibers constituting the fibrous structure may acquire a straightness over distances of 5 µm or more, 10 µm or more or even 20 µm or more. In parallel or in addition to this straightness, a majority of the fibres (i.e. 50% or more) constituting the fibrous structure tends to become cross-link free, i.e. not cross-linked to neighboring fibers. The majority of the fibres is e.g. substantially cross-link free with respect to neighboring fibers at their contact points. According to embodiments of the present invention, fibrous structures are obtained that comprise fibres that are cross-link free and thus not linked to each other, i.e. wherein the majority of the fibres, e.g at least 50%, advantageously at least 70%, more advantageously at least 90%, even more advantageously 95% remains independent. Cross link free thereby may be less than 1 cross link per 1 mm fiber length, advantageously less than 1 cross link per 5 mm fiber length, more advantageously less than 1 cross link per 1 cm fiber length, still more advantageously less than 1 cross link per 5 cm fiber length, even more advantageously without cross links over the full length of the fibre. This effect is particularly pronounced for outlets separated by 4 cm or more. When three or more outlets are used, the outlets (e.g. needles) are advantageously arranged in sets of triangles (see FIG. 5) with a distance between each outlet of minimum 1 cm and maximum 100 cm, more advantageously of minimum 4 cm and maximum 100 cm and most advantageously of minimum 8 cm and maximum 100 cm. In embodiments of the present invention where very volatile and/or easily ionizing solvents are used, the positioning of the needles may be adapted as shown in FIG. 6. In FIG. 6, the same individual positioning of the needles is respected as shown in FIG. 5 but for each two lines of needles, a third line is removed. In that case an individual needle is never surrounded by needles at all sides. This permits an easier evaporation of the solvent from the fibre formation area. The purpose a needle set-up as shown in FIG. 6 is to avoid favouring electrical discharges when using volatile or ionizing solvents. The total number of outlets is not limited to a maximal value. For instance, the total number of outlets used in a configuration may be between 2 and 20000. Advantageously, the total number of outlets, e.g. needles, used in a configuration is between at least 3 and 500 (see FIG. 5). Different rows, such as e.g. neighbouring rows, of outlets may be parallel but shifted with respect to the corresponding position of the outlets with respect to each other. The latter may be evaluated with respect to the average direction of the relative movement of the receiving surface. The configuration of the outlets may be such that the outlets are positioned in triangular shaped groups of outlets.

The electrospinning device according to the present invention comprises also a receiving surface. The receiving surface is facing the set of outlets. The receiving surface is a surface such as but not limited to a plate (e.g. a metallic plate), a foil or textile structure. The receiving surface may optionally be coated with a perforated or non-perforated layer, e.g. a perforated or non-perforated polymer/plastic layer. The receiving surface may be a planar part of a larger surface not necessarily planar in all its parts. For instance, the receiving surface may be part of a larger belt comprising winded parts. The surface may contain a liquid surface on which the fibers are deposited. The receiving surface is adapted for receiving output from the set of two or more outlets. The receiving surface may take any spatial orientation. For instance, it may be horizontal with the set of outlets above the receiving surface or with the receiving surface above the set of outlets. In those cases, the outlets would therefore be oriented downward or upward respectively. For instance the outlets (e.g. needles) are positioned in a lower plate and solution or melt (e.g. polymer solution or melt) jets move upwards the device. The receiving plate may also be oriented vertically. Other orientations for the receiving plate are of course possible (e.g. at 45° or any other angle with the horizon). The ensemble of, on one hand, the outlets and on another hand the receiving surface is also referred to as a spinneret. At least one of the receiving surface and the set of outlets is adapted to be moveable, i.e. one or more relative movements may be provided between the receiving surface and the set of outlets. Preferably, at least one of these relative movements is in one direction parallel to the receiving surface and is responsible for the lengthwise growth of the fibrous structures. Preferably, this relative movement is caused by a movement of the receiving surface itself. The direction in which the set of outlets may be adapted to move in embodiments of the present invention, can be either parallel to the receiving surface or perpendicularly to the receiving surface. The movement of the outlets can also be a combination of a movement parallel to the receiving surface and perpendicular to the receiving surface. In embodiments of the present invention, the movement of the outlets is advantageously a reciprocal movement, e.g. a movement between two fixed points. This reciprocal movement is preferably parallel to the receiving surface and perpendicular to the direction of the movement responsible of the lengthwise growth of the fibrous structure. The movement of the receiving surface may be parallel to said receiving surface, orthogonal to said receiving surface or a combination of both. Advantageously, in embodiments of the present invention, the receiving surface can move continuously in one direction parallel to said receiving surface. Advantageously, the device is adapted for providing a relative movement to the set of outlets and the receiving surface, the relative movement being e.g. a combination of a relative movement in a first direction parallel to the receiving surface and in a second direction also parallel to the receiving surface but different from said first direction. For instance, the receiving surface can be adapted to undergo a relative movement at an angle to the first direction such as optionally substantially perpendicular to said first direction. Said first and second direction can be perpendicular to each other and parallel to said receiving surface. Advantageously, the set of outlets and the receiving surface can move relatively to each other so that the set of outlets moves in a first direction parallel to the receiving surface (e.g. the y-direction, see FIG.2), e.g. reciprocally such as e.g. between two inversion points, and the receiving surface moves continuously in a second direction perpendicular to the first direction (e.g. the x-direction, see Fig.2) but in the plane of said receiving surface. This type of reciprocal movement of the outlets is advantageous because it allows overlapping the output of the outlets as received on the receiving surface from the different outlets. The output of an outlet as received on the receiving surface may be referred to as the fibre umbrellas on the receiving surface. The fibre umbrellas have a high tendency to reject each other due to their charge and do not easily overlap if the configuration is used as a stationary system, i.e. if there is not at least a reciprocal relative movement between the receiving surface and the set of outlets. The amount of relative reciprocal movement may be selected such that the output of neighbouring outlets at least overlaps. Additionally, the width of the obtained fibrous structure can be increased in this way, i.e. by using a reciprocal movement. The set of outlets is advantageously subject to a relative reciprocal movement with respect to the receiving surface with an average speed between 0.1 cm s⁻¹ and 100 cm s⁻¹ in the direction of the lengthwise growth of the fibrous structure. Further relative movement, preferably a continuous relative movement in one direction parallel to the receiving surface, between the outlets and the receiving surface allows continuous production of larger fibrous structure surface areas, i.e. such a relative movement is responsible for the lengthwise growth of the fibrous structures. In this respect, the receiving surface is advantageously moveable with a speed between 10 cm h⁻¹ and 100 m h⁻¹.

The electrospinning device of the present invention further comprises a voltage source adapted to apply a potential difference between the outlets and the receiving surface. The voltage source may be a DC-high voltage source able to apply a potential difference selected in the range between 100 and 200000 V over the spinneret, i.e. between the outlets and the receiving surface. For instance, the outlets (e.g. needles) may be electrically in contact with each other through a conductive (e.g. metallic) plate or holding structure. In other embodiments, a semi or non-conductive first material plane (e.g. a plate) or holding structure can be used in combination with means such as e.g. a metallic wire for electrically connecting all the outlets (e.g. needles). The voltage source may be connected to an electroconductive structure comprising the outlets or to means (e.g. wire) for electrically connecting all the outlets (e.g. needles). The receiving surface is advantageously grounded. Optionally it can be used ungrounded (floating) but adapted security measures are then preferably taken. Alternatively, the receiving surface can also be set at a certain potential using a second DC voltage source.

The electrospinning device of embodiments of the present invention further may comprise at least one recipient for containing a solution or melt to be electrospun from said outlets. The recipient may contain a polymer solution or melt. Alternatively, the receipients may be external to the electrospinning device.

The electrospinning device of embodiments of the present invention advantageously further comprises means for providing the solution or melt to the outlets. The means for providing the solution or melt to the outlets can be any means known by the person skilled in the art. Examples of means for providing the solution or melt to the outlets comprise but are not limited to pumps or syringes among others as well as transfer means such as e.g. tubes.

For instance, each outlet (e.g. needle) can be fed with a solution or melt (e.g. a polymer solution or melt) by an individual means (such as e.g. an individual peristaltic pump). In some embodiments, a multichannel means (such as e.g. a multichannel peristaltic pump) can be used in which each channel feeds one individual outlet. Also a multiple of multichannel means (e.g. pumps) can be used, dependent on the amount of outlets that need to be fed with polymer solution or melt. In other embodiments, an anesthesia type pump can be used to feed the outlets (e.g. needles) through syringes filled with polymer solution or melt and positioned in the anesthesia pump. Alternatively, the outlets can be fed with solution or melt from a central tank kept at a predetermined, e.g. constant pressure with pressure valves and/or pressurized air. In some embodiments, a multiple amount of outlets (e.g. needles) can be fed by one source e.g. a peristaltic or anesthesia pump. The injection rate (e.g. the pump rate) of solution, e.g. polymer solution, or melt per outlet (e.g. needle) may be between 0.01 and 500 mL h⁻¹.

Solutions or melts usable within the present invention are any solution or melt known by the person skilled in the art to be suitable for forming fibers by electrospinning. The solution or melt can be obtained from polymers. Suitable polymers comprise but are not limited to polyamides, polystyrenes, polycaprolactones, polyacrylonitriles, polyethylene oxides, polylactic acids, polyacrylic acids, polyesteramides, polyvinyl alcohols, polyimides, polyurethanes, polyvinylpyrrolidon, collagen, cellulose and related products, chitosan, methacrylates, silk and combination thereof. The solution or melt may also contain metallic particles or metals dissolved as metallic ions so that metal containing fibers can be formed.

As an optional feature, the solutions or melts may contain an additional compound, such as compounds with antibacterial, pharmaceutical, hydrophobic/hydrophilic, anti corrosion, catalytic, oxidative/reductive and other properties.

The electrospinning device of the present invention may optionally further comprise a surrounding element, i.e. an element surrounding the other elements of the electrospinning device. For instance, the surrounding element can form a jacket around the spinneret and prevents the spinneret from instability such as air turbulence and/or allow solvent recuperation. Air turbulence are advantageously avoided in the spinneret because it may cause instability in the melt or solution jets and the fibre umbrellas produced by those jets on the receiving surface. The surrounding element may for instance be composed of plates of a non-conductive material connected to each other to form an enclosure.

The electrospinning device of the present invention may further comprise one or more optional temperature control means/systems. Those temperature control means may be added to the electrospinning device for instance in order to obtain higher reproducibility in fibre production. Fluctuations of temperature can have its influence on the evaporation rate of the solvent and thus on the final dimensions of the fibres and the porosity of the structures. Temperature controlling means are therefore advantageous. The solution or melt in the recipient may be temperature conditioned by using containers for (e.g. a liquid bath such as an oil or water bath) temperature control. The control of the temperature can also be operated during the solution transport from the recipient to the outlets via jacketed tubes that are connected directly or indirectly with a cooling/heating system such as said containers for temperature control. The spinneret may be temperature controlled by using means for bringing heated/cooled air in the spinneret. For instance, the electrospinning device of the present invention may comprises a temperature control system that allows to control the temperature in the range 280-1500 K.

The electrospinning device of the present invention is adapted for providing a predetermined distance profile between the outlets (5) and the receiving surface (8) during production of the fibrous structure for inducing a predetermined fibre diameter profile along a dimension of the electrospun fibrous structure. The predetermined fibre diameter profile may be obtained in the thickness dimension of the electrospun fibrous structure. The latter allows to obtain an electrospun structure comprising fibres, wherein the diameter of the fibres in one direction of the electrospun fibrous structure has a predetermined profile. The latter may be advantageous as it provides to control certain properties of the electrospun fibrous structure in this direction. The predetermined distance profile may for example be providing a decreasing or increasing distance between the outlets (5) and the receiving surface (8) along said first direction, although the invention is not limited thereto. In one example, the predetermined distance profile may be providing a monotonously decreasing or increasing distance between the outlets (5) and the receiving surface (8). This feature permits to obtain an electrospun structure comprising fibres, wherein the diameter of said fibres decreases, e.g. monotonously decreasing, along a dimension of said electrospun fibrous structure. This can be realised in various not mutually excluded alternative ways as will be described herebelow. Providing a predetermined distance profile, e.g. (monotonously) decreasing or increasing distance, between the outlets (5) and the receiving surface (8) along the direction of lengthwise growth of the fibrous structure can be achieved by moving the set of outlets and the receiving surface relatively to one another at least with a component in a direction perpendicular to the receiving surface (see first embodiment below and FIG. 2), e.g. during electrospun operation, or by placing the outlets above the receiving surface according to an, optionally fixed, predetermined distance profile. For example in a decreasing or increasing fibre thickness profile, the outlets may be positioned in such a way that the outlets further away in the direction of lengthwise grow of the fibrous structure are also closer to the receiving surface (see FIG. 3 and 4). An obvious alternative is to place the outlets above the receiving surface in such a way that the outlets further away in the direction of lengthwise grow of the fibrous structure are also further away from the receiving surface. As will be shown this may be done by introducing a distance variation between individual outlets as well as by introducing a distance variation between different sub-groups of outlets. Alternatively, also the receiving surface can move to change the distance or positioned under a certain angle to obtain a predetermined distance profile, e.g. an increasing or decreasing outlet to receiving surface distance, e.g. monotonously.

A first embodiment to provide a predetermined distance profile, e.g. a decreasing or increasing distance, between the outlets and the receiving surface is to move vertically, and preferably continuously, the whole set of outlets relatively to the receiving surface (or to move vertically the receiving surface relatively to the set of outlets) during the fibre production. In this embodiment, it is necessary that the receiving surface carrying the growing fibrous structure is re-exposed during a longer period or repeatedly to the outlets in order to build the fibrous structure with varying fibre diameter in the thickness direction of the fibrous structure according to a predetermined profile. The fibrous structure is therefore only collected after a sufficiently long exposure or after that a sufficient number of re-expositions occurred. Re-exposition is easily achieved if an endless belt is used. Otherwise, a reciprocal movement of the receiving surface in the X direction of figure 2 may be used, in order to create large fibrous structures while coping with the limited size of the electro-spun system. If the vertical relative movement of the receiving surface and the set of outlets is discontinuous, a layered fibrous structure will be produced wherein each subsequent layer is composed of fibres having an average diameter different from (e.g. lower than) the previous layer. If this movement is continuous, the average diameter of the produced fibres continuously decreases (or increase) along one dimension (e.g. the thickness) of the fibrous structure. The variation of the fibres diameter in any section perpendicular to said dimension, may be limited, e.g. below 10%. In systems whereby the fibrous structure is moving during displacement of the outlets in the vertical direction with respect to the receiving surface, the variation of the diameter in a section perpendicular to the thickness dimension depends on the speed of movement. The slower the movement of the receiving surface, the smaller the variation over a given surface will be.

Some examples for inducing a fibre thickness profile are moving the set of outlets perpendicularly (e.g. in the z direction, see FIG.2) to said receiving surface, moving the receiving surface vertically (e.g. in the z direction, see FIG.2) towards or away from the set of outlets or both, moving the set of outlets and the receiving surface towards each other or away from each other. The distance between the outlets and the receiving surface can advantageously be varied between 1 and 100 cm. This first embodiment enables to implement a fluctuation of the average fibre diameter as a function of thickness of the obtained fibrous structure. As the fibrous structure is formed by exposing it long time in the electrospun system or by re-exposing it, the system gives rise to batch type processing.
In Fig. 2, an example of electrospinning device according to this first embodiment to provide a predetermined distance profile, e.g. an optionally monotonously, decreasing or increasing distance between the outlets and the receiving surface is presented together with geometrical axes x, y and z. The z axis is the vertical axis while the x and the y axis defines two horizontal axis perpendicular to each other. This device comprises a high voltage source **1** and a pump **2** (e.g. a peristaltic pump, an anesthesia pump or a container kept under constant pressure with pressurized air). The device also comprises an upper element **7** with a set of outlets 5 (here needles) which are positioned horizontally in a planar fashion. The device also comprise a receiving surface **8** adapted to repeatedly move in the X direction (an endless belt). The device further comprises means **11** for transferring/providing a solution or melt to the outlets and means **10** for providing a relative movement (here a monotonous vertical movement in the Z direction and a reciprocating movement in the Y direction) to the set of outlets **5** with respect to the receiving surface **8.** The device is surrounded by a surrounding element **9** (here transparent). The device further comprises evacuation means **15** to remove solvent. The evacuation means can be connected to a chimney or to a solvent recuperation system. In the example of FIG. 2, the high voltage source **1** is a DC-source able to apply a potential difference between 100 and 200.000 V over a spinneret, said spinneret consisting of two elements **7** and **8** arranged in parallel against each other. The upper element **7** is a plate comprising a certain amount of holes in which metallic needles **5** are positioned. The needles are electrically in contact with each other through the metallic plate **7.** In another setup a semi or non-conductive upper plate **7** can be used in combination with a conductive (e.g. metallic) wire connecting all the needles **5.** The high voltage source **1** is connected to the upper plate **7,** when electroconductive, or to the wire that interconnects all needles **5.** The lower plate **8** is either a metallic plate, foil or textile structure, which optionally can be coated with a perforated or non-perforated polymer/plastic layer. This plate is grounded. Optionally it can be used as ungrounded (floating) but this can cause unsafe situations. In another embodiment the upper and lower plate are inverted, thus the needles are positioned in the lower plate and polymer jets move upwards the device.

The device depicted in Fig.2 can be operated as follows: A voltage is set between the outlets **5** and the receiving surface **8.** A liquid or melt to be electrospun is transferred from a recipient to the outlets **5** via the transfer means **11** (here a flexible tube) by the action of means **2** for providing a solution or melt to the outlets. In order to induce a distance profile between the outlets and the receiving surface during electrospinning operation, the relative movement can be obtained by moving the outlets (and therefore also here the upper plate) in the Z direction by the operation of movement means **10** for moving the set of outlets, or for moving the receiving surface. It is this movement that allows a predetermined profile of the fibre diameter variation along the thickness of the obtained fibrous structure (e.g. a mat). The distance between the outlets and the receiving surface can preferably be varied between 1 and 100 cm. The actual border values that will be used depend on the specification of the product to be obtained. Simultaneously, the endless belt **8** is accumulating the fibrous structure formed. In this way, a predetermined distance profile, e.g. an, optionally monotonously, decreasing or increasing distance between the outlets and the receiving surface, while the receiving surface is moved relatively to said outlets in one direction parallel to said receiving surface, can be obtained. Simultaneously, the upper plate 7 comprising the outlets is moved reciprocally in the Y direction between two inversion points in order to assure a good overlap of the solution or melt output (also called nanofibre umbrellas). Those umbrellas have a tendency to reject each other, which is detrimental to their overlap in the absence of reciprocal movement in the Y-direction. This reciprocal movement is therefore particularly preferred. Additionally, the use of a reciprocal movement in the Y-direction permits to increase the width of the nanofibrous structures. The movement of the receiving surface 8 allows the production of large nanofibrous structure surface areas.

The device of FIG.2 permits the production of fibrous structures wherein the fibre diameter varies according to a predetermine profile, e.g. monotonously along the thickness of the obtained fibrous structure, although the invention is not limited thereto. The predetermined profile of the fibre diameter may for example also be a larger diameter at the surfaces of the fibrous structure, a smaller diameter at the surfaces of the fibrous structure or any other desired profile. The diameter variation obtained can be both continuous or discontinuous. If discontinuous, the fibrous structures produced will appear layered. This first embodiment is not adapted for the continuous production of fibrous structures. The two next embodiments advantageously permit the continuous production of fibrous structures according to the present invention, which is often preferred over batch production.

A second embodiment to provide a predetermined distance profile, e.g. an, optionally monotonously, decreasing or increasing distance between the outlets and the receiving surface is to arrange a plurality of outlet sets along the direction of the lengthwise production of said fibrous structures, wherein the outlets are arranged in the lengthwise production of the fibrous structure according to a predetermined profile. For example, each outlet set is at a distance to the receiving surface lower than the next outlet set along said lengthwise direction (see FIG.3), which would result in a decreasing or increasing profile, e.g. monotonously increasing or decreasing profile. An obvious alternative for the particular example of increasing or decreasing profile is of course to arrange a plurality of outlet sets along the direction of the lengthwise growth of said fibrous structures, wherein each outlet set is at a distance to the receiving surface higher than the next outlet set along said direction. Those two alternatives have the advantage that they allow the continuous production of large nanofibrous structure surface areas while the embodiment of FIG. 2 only permits the batchwise production of fibrous structures.

In FIG.3, an example of an electrospinning device according to this second embodiment to provide a predetermined profile, e.g. an, optionally monotonously, decreasing or increasing distance between the outlets and the receiving surface is presented together with geometrical axes x, y and z. The z axis is the vertical axis while the x and the y axis defines two horizontal axis perpendicular to each other. This device is composed of two outlet sets **5,** each connected to a high voltage source **1** and to a pump **2** (here hidden in a box), which are positioned horizontally in a planar fashion. The device also comprises a receiving surface **8** (an endless belt) adapted to move in the X direction below both sets of outlets. The system also comprises means **11** for transferring/providing a solution or melt to the outlets. Means **10** for providing a movement of the set of outlets **5** with respect to the receiving surface **8** are here not necessary but could be provided additionally. Such means **10** could be useful to adapt the distance between each set of outlets and the receiving surface to the specific fibrous structure to be produced. The electrospinning device of FIG. 3 is particularly well suited to continuous production, particularly to the continuous production of layered fibrous structures. In other words, the number of layers with different fibre diameters in the laminated structure determines the number of modules (outlets sets) necessary, which in principle is unlimited (FIG. 3 shows a device comprising two modules). In addition, the use of a range of modules connected to each other contributes positively to the high-throughput production possibilities of such laminated nanofibrous structures.

In operation, the device depicted in FIG.3 operates as follows: A voltage is set between each set of outlets **5** and the receiving surface **8.** A liquid or melt to be electrospun is transferred from a recipient to each of the set of outlets **5** via the transfer means **11** (here a flexible tube) by the action of means **2** for providing a solution or melt to the outlets. The receiving surface is moved continuously in the X direction while collecting the fibrous structure formed from said receiving surface. While progressing in the X direction, the receiving surface is exposed to the output of outlets, e.g. monotonously, closer to it. Simultaneously, the outlets are moved reciprocally in the Y direction to give a good overlap of the outputs of the outlets on the receiving surface.
A third embodiment to provide a predetermined distance profile, such as for example a decreasing or increasing distance profile, between the outlets and the receiving surface is to arrange the outlets in such a way that the outlets are comprised in a plane not horizontal relatively to the receiving surface. While in the device of the second embodiment to provide a predetermined distance profile, for example decreasing or increasing distance, between the outlets and the receiving surface (see FIG. 3), the fibrous structures obtained are layered and at the interface between two layers the diameter of the fibres changes in a discrete way, in the third embodiment to provide a predetermined distance profile, such as for example decreasing or increasing distance, between the outlets and the receiving surface, fibrous structures can be obtained wherein the change in diameter within a dimension of the fibrous structure-is smoother, e.g. a continuous variation of the diameter across the thickness of the produced fibrous structure can be obtained. In one example, the outlet sets are arranged in such a way that the outlets are comprised in a plane not horizontal to the receiving surface is to incline the set of outlets (e.g. the upper plate comprising them) at an angle between 5 and 50° relatively to the receiving surface (often relatively to the horizontal). This results in a continuously increasing or decreasing outlet (e.g. needle tip) to receiving surface distance (for each row of needles) along the x-direction, i.e. along the direction of the lengthwise growth of the fibrous structure. Preferably, each outlet is oriented perpendicularly to the receiving surface despite said angle, although the invention is not limited thereto. An example of this third embodiment to provide a predetermined distance profile between the outlets and the receiving surface is schematically presented in FIG. 4. With this setup laminated nanofibrous structures can be continuously produced that show a smooth profile of the average nanofiber diameter as a function of depth (FIG. 7), while for the setup of FIG. 3. only discrete changes of the nanofiber diameter are obtained at the interfaces between the individual layers.

In Fig. 4, an example of electrospinning device according to this third embodiment to provide a predetermined distance profile between the outlets and the receiving surface is presented together with geometrical axes x, y and z. The z axis is the vertical axis while the x and the y axis defines two horizontal axis perpendicular to each other. This device is composed of two planar outlet sets **7,** each connected to a high voltage source **1** and to a pump **2** (here hidden in a box), which are, in the present example, positioned slantwise to the receiving surface **8.** It is to be noticed that an alternative distance profile also may be applied. The receiving surface **8** is adapted to move in the X direction below both sets of outlets. The system also comprises means **11** for transferring/providing a solution or melt to the outlets. Means **10** for providing a movement of the set of outlets **5** with respect to the receiving surface **8** are here not necessary but could be provided additionally. Such means **10** could be useful to adapt the slope of the planar outlet sets **7** in order to create different variation of the distance between each set of outlets and the receiving surface. This adaptation permits different specific fibrous structure to be produced with the same device.

In operation, the device depicted in FIG.4 operates as follows: A voltage is set between each set of outlets **5** and the receiving surface **8.** A liquid or melt to be electrospun is transferred from a recipient to each of the set of outlets **5** via the transfer means **11** (here a flexible tube) by the action of means **2** for providing a solution or melt to the outlets. The receiving surface is moved continuously in the X direction while collecting the fibrous structure formed. While progressing in the X direction, the receiving surface is exposed to the output of outlets position at a different distance, e.g. closer to it. Simultaneously, the outlets are moved reciprocally in the Y direction to give a good overlap of the outputs of the outlets on the receiving surface.

In some embodiments, the electrospinning device of the present invention comprises movement means for moving the set(s) of outlets and/or said receiving surface, such as but not limited to one or more motors and one or more actuation means, such as e.g. transmission axis. The movement means may be adapted for inducing one or more of the relative movements as described above.

The device may comprise a controller for controlling said movement means and therefore for controlling the movement of the outlets and the receiving surface during the production process of the fibrous structure or for setting the distance and/or the slope of each set of outlets according to the target fibrous structure.

In a second aspect, the present invention relates to a method for producing fibrous structures. This method comprises the steps of providing a set of outlets for outputting solution or melt, providing a receiving surface for receiving output from said set of outlets, moving said receiving surface in a first direction parallel to said receiving surface, applying a potential difference, i.e. a voltage between said set of outlets and said receiving surface, during said moving and applying, providing a solution or melt to the outlets. Preferably, the distance between the outlets and the receiving surface is according to a predetermined profile, in order to obtain a predetermined fibre thickness profile over the fibrous structure. The predetermined profile may be an optionally monotonously, decreasing profile along said first direction. This profile may be obtained because of the geometry of the system (e.g. embodiments of FIG. 3 and 4) or because of an actual relative movement of the set of outlets relatively to the receiving surface. The method may advantageously be performed with a system as described in the first aspect. The potential difference may be selected in the range between 100 and 200000 V. The movement step may be performed by actuating means for further moving said set of outlets and/or said receiving surface to generate a good filling of the fibrous structure. As a result, at least one of the receiving surface and the set of outlets is further moved. The direction in which the set of outlets may further be moved can be parallel to the receiving surface, perpendicular to the receiving surface or a combination of both. The further movement of the outlets may be a reciprocal movement, e.g. a movement between two fixed points, preferably parallel to the receiving surface and perpendicular to the direction of the lengthwise growth of the fibrous structures. The direction in which the receiving surface may further move can be parallel to said receiving surface, orthogonal to said receiving surface or a combination of both. Advantageously, the receiving surface is further moved continuously in one direction parallel to said receiving surface. Advantageously, the set of outlets is further moved reciprocally in a first direction parallel to the receiving surface and the receiving surface is further moved in a second direction parallel to the receiving surface but different from said first direction. For instance, the receiving surface can be further moved at an angle to the first direction such as optionally substantially perpendicular to said first direction. Said first and second direction may be perpendicular to each other and parallel to said first plane and said receiving surface. Advantageously, the set of outlets and the receiving surface are further moved relatively to each other so that the set of outlets moves along the y-direction (see for instance FIG.2, FIG.3 or FIG.4) between two inversion points and the receiving surface further moves continuously in a direction perpendicular to the y-direction (e.g. the x-direction in FIG.2, FIG.3 or FIG.4) but in the plane of said receiving surface. The set of outlets may further move with an average speed between 0.1 cm s⁻¹ and 100 cm s⁻¹. The receiving surface may move with a speed between 10 cm h⁻¹ and 100 m h⁻¹.

The solution or melt may be kept in a recipient which may but does not have to be temperature controlled. Providing the solution or melt can be performed by solution or melt actuating means for providing the solution or melt to the outlets. Those means (such as e.g. a pump) transfer the solution or melt to the outlets via transfer means which may but do not have to be temperature controlled. Once at an outlets, the solution or melt forms a droplet from which a filament will be drawn and projected toward the receiving surface under the action of the potential difference. The receiving surface acts therefore as a collecting surface. The shape of the jet of solution or melt leaving an outlet is usually conical and forms a so-called umbrella, i.e. a covered area on the receiving surface. In an advantageous embodiments of the present invention, due to a reciprocal lateral relative movement of the outlets toward the receiving surface, the umbrella overlaps and form a fibrous structure such as a mat composed of fibres. The fibrous structures can in a later stage be recovered from the receiving surface by any method well known to the person skilled in the art.

In a third aspect, the present invention relates to a fibrous structure. A first embodiment of a fibrous structure according to the present invention shows a number of advantages and innovative aspects when compared to the commonly described nanofibrous structures of the prior art. These features are obtained through the specificity of the used electrospinning devices according to the first aspect of the present invention. The fibrous structures of the present invention shows a variation of the diameter of its individual fibres along a dimension of the fibrous structure, e.g. across the thickness of the fibrous structure. In an embodiment, the present invention relates to an electrospun fibrous structure comprising fibres, wherein the diameter of said fibres varies according to a predetermined profile, e.g. decreases or monotonously decreases along a dimension of said electrospun fibrous structure and wherein the variance of the fibres diameter in any section perpendicular to said dimension may be below 10%.. In an embodiment, the electrosopun fibrous structure of the present invention is a laminated structure composed of layers of nanofibres, each subsequent layer being composed of fibres having an average diameter lower than the fibres of the previous layer. The average diameter of the fibres is therefore varying according to a predetermined profile, e.g. decreasing or increasing monotonously, across the thickness of the electrospun fibrous structure.

The electrospun fibrous structures of the present invention can be cut in any desired shape dependent on the requirements of the envisaged applications. The surface area can vary from 5 mm² to 10 m², the thickness from 100 nm to 30 cm and the diameter of the individual fibres from 3 nm to 5 µm. In an embodiment, the electrospun fibrous structure of the present invention is porous. The electrospun fibrous structures have preferably a porosity of at least 65%. The pore sizes can vary from 30 nm to 8 µm.

As an advantageous feature, the electrospun fibrous structure of the present invention may comprise a majority, i.e. 50% or more of straight fibers. In one embodiment, the fibrous structure forms a mat. The straightness of the fibres can for instance be inferred from an image analysis. Preferably, the majority of the fibers (i.e. 50% or more) comprised in the fibrous structure are straight, i.e. consists of a majority of segments (i.e. 50% or more) substantially straight over a distance of 5 µm. By substantially straight, it must be understood that the major axis of the fibre, i.e. along the direction of the fibre, changes over an angle less than 45°, e.g. less than 30°, or e.g. less than 15° or e.g. less than 5°, considering a distance of 10 micrometer over which the angle change was measured. This angle is the largest angle which can be measured between tangents at two points of the major axis over the length of the fiber considered. The standard deviation to linearity over the distance in question may be not exceeding 5%.

As an advantageous feature, the fibrous structures of the present invention may comprise only few or no crosslinking, e.g. microfibrous or nanofibrous structure wherein a majority of the fibers (i.e. 50% or more) comprised are substantially cross-link free. The fibrous structure is an electrospun fibrous structure, it is a structure made by electrospinning. They are advantageously not cross-linked to neighboring fibers. Cross-linking thereby means that a link occurs between two fibres, not just that two fibers are touching. This is the result of the spacing between the outlets being at least 1 cm. Without being bound by theory, it is believed that this effect is due to an easier and therefore faster evaporation of the solvent during the fibres formation. It is believed that for spacing between the outlets inferior to 1 cm, the solvent takes too much time to evaporate during the fibres formation. This leads to fusing of adjacent fibres and therefore to crosslinks. If the fibrous structure is made from a melt, the problem may be an incomplete elimination of the heating effect occurring when outlets are too close to each other. The fiber formation then is not complete and a sort of intermediate phase between melt and solid then may be present, allowing formation of cross-linked fibres. Another advantageous feature of the fibrous structures obtained is that they have a porosity of at least 65%, advantageously between 65 and 99%.

In embodiments, the present invention also relates to a fibrous structure wherein the thickness of the fibres is uniform, i.e. the standard deviation of the thickness throughout the fibrous structure does not exceed 80%, advantageously 50%, most advantageously 20%

The present invention also relates to a fibrous structure comprising more or all of the above identified properties. As an optional feature, the fibrous structures according to the present invention can be made comprising a majority of fibers (i.e. 50% or more) randomly oriented, i.e. not oriented in a particular direction (e.g. not aligned). The last effect is helpful in achieving an increased porosity. In embodiments where the receiving surface moves continuously in one direction, this effect can be obtained for example by choosing a speed for the receiving surface between 10 cm h⁻¹ and 100 m h⁻¹.

As an optional feature, the diameter of a majority of the fibres (i.e. 50% or more of the fibers) comprised in the fibrous structures of the present invention have a diameter of 3 nm or higher, advantageously 10 nm or higher. As an optional feature, the diameter of a majority of the fibres (i.e. 50% or more) comprised in the fibrous structures of the present invention have a diameter of 2000 nm or lower, advantageously 800 nm or lower, most advantageously 700 nm or lower. When the fibers have an average diameter of 800 nm or lower, they will be referred to as nanofibers and the fibrous structures made therefrom as nanofibrous structures. As an optional feature, the diameter of a majority of the fibers (i.e. 50% or more) comprised in the fibrous structures of the present invention have a diameter of 3 to 2000 nm, advantageously between 10 and 2000 nm, advantageously between 3 and 800 nm, more advantageously a diameter of 10 to 700 nm.

As can be seen from the examples the fibre diameter is dependent on the distance between the outlets and the receiving surface. The profile of the relationship between the fibre diameter and the distance may be polymer and solvent specific. Therefore a profile can be determined after studying the polymer solution or melt because it is polymer and solvent specific. It can be determined via trial and error, via experimental results, via a theoretical model, etc. As another optional feature, the fibrous structures obtained have a width between 15 and 10000cm.

In embodiments of the third aspect of the present invention, the fibrous polymeric structures have a porosity of at least 65% and a width comprised between 15 and 10000 cm.

The method of the second aspect applied to the device of the first aspect permits to obtain fibrous structures having outstanding properties, and remarkable property being the variation of the fibers diameter across a dimension of the fibrous structure.

In some embodiments of the third aspect, the fibrous structures are obtained laminated, i.e. multi-layered. Advantageously, the average fibre diameter is different for each pair of adjacent layers within the fibrous structure. This may be achieved by using a different distance between the set of outlets and the receiving surface for each layer (see e.g. FIG. 3). The obtained laminated fibrous structures have a number of advantages compared to their non-laminated counter parts. Firstly, the combination of layers with small fiber diameter and layers with somewhat bigger fibers improve on the overall strength of the fibrous structure. Secondly, the absorption/release properties of the fibrous structure can be optimized as a function of application and this in a single production step and finally, multitasking and multifunctionality can be obtained by using a laminated structure, such as multilevel filtration in one single multilayered structure.

It is to be understood that although preferred embodiments, specific constructions and configurations, as well as materials, have been discussed herein for devices according to the present invention, various changes or modifications in form and detail may be made without departing from the scope and spirit of this invention. For example, steps may be added or deleted to methods described within the scope of the present invention. Whereas the present invention has been described with respect to a method for manufacturing, an electrospinning device and the resulting fibrous structures, the present invention also relates to a controller for controlling a relative distance between the outlets and the receiving surface for generating different properties between different layers in a fibrous structure.

### Example 1

Polyester amide (PEA) with molecular weight of about 20.000 g mol⁻¹ was dissolved in chloroform to obtain a solution of 25% PEA. The solution was pumped to a set of 24 outlets with a multitude of multichannel peristaltic pumps, using a flow rate of 15 mL h⁻¹ per outlet. In the spinneret an electrical field of about 1000 V cm⁻¹ is applied over the outlets and the receiving surface in order to allow electrospinning of the polymer solution. The outlets were positioned in the triangle configuration of 4 rows of 6 outlets per row. Temperature control was performed at 298 K. The outlet surface was positioned under an angle of 10° relative to the receiving surface and the outlet surface moved perpendicular to the movement of the receiving surface. The speed of the receiving surface was 40 cm h⁻¹, while the rate for the outlet surface is 1 cm s⁻¹. After 2 hours of spinning a nanofibrous structure of 300 µm thick was obtained with a length of about 1.5 m and a width of 80 cm. The average nanofibre diameter changed as a function of depth from 500 nm (FIG. 8) at one side of the structure to 300 nm (FIG. 9) at the other side. The side with the largest diameters corresponds to the fibers obtained from the outlets positioned the closest against the receiving surface, while the smallest diameters (at the other side of the nanofibrous structure) were obtained from the outlets having the largest distance from the receiving surface. FIG. 10 shows the relationship for nanofibre diameter and distance between outlets and receiving surface.

### Example 2

Poly amide 6/6 (PA66) with molecular weight of about 20.000 g mol⁻¹ was dissolved in formic acid to obtain a solution of 14% PA66. The solution was pumped to 2 sets of each 24 outlets with a multitude of multichannel peristaltic pumps, using a flow rate of 2 mL h⁻¹ per outlet. In the spinneret an electrical field of about 3.500 V cm⁻¹ was applied over the outlets and the receiving surface in order to allow electrospinning of the polymer solution. The-outlets were positioned in the triangle configuration of 4 rows of 6 outlets per row. Two spinnerets were used, each operational at a different distance between the outlets and the receiving surface. Temperature control was performed at 298 K. The first outlet surface was positioned at a distance of 4 cm, while the second was positioned at a distance of 6 cm from the receiving surface. The speed of the receiving surface was 60 cm h⁻¹, while the rate for the outlet surface is 1 cm s⁻¹. After 2 hours of spinning a nanofibrous structure of 100 µm thick was obtained with a length of about 1.2 m and a width of 80 cm. The average nanofibre diameter changed in one step as a function of depth from 285 nm (FIG. 11) at one side of the structure to 180 nm (FIG.12) at the other side. The side with the largest diameters corresponds to the fibers obtained from the outlet surface positioned at 4 cm from the receiving surface, while the smallest diameters (at the other side of the nanofibrous structure) are obtained from the outlet surface positioned at 6 cm from the receiving surface.
FIG. 13 shows the profile of the distance between the outlets and the receiving surface and the average nanofibre diameter, obtained using the processing setup as described in example 1. This profile is plotted for different concentrations of PA66.

### Example 3

Cellulose acetate (CA) with molecular weight of about 30.000 g mol⁻¹ was dissolved in acetone/Dimetylacetamide 2:1 to obtain a solution of 14% CA. The solution was pumped to 2 sets of each 24 outlets with a multitude of multichannel peristaltic pumps, using a flow rate of 10 mL h⁻¹ per outlet. In the spinneret an electrical field of about 850 V cm⁻¹ was applied over the outlets and the receiving surface in order to allow electrospinning of the polymer solution. The outlets were positioned in the triangle configuration of 4 rows of 6 outlets per row. Two spinnerets were used, each operational at a different distance between the outlets and the receiving surface. Temperature control was performed at 298 K. The first outlet surface was positioned at a distance of 20 cm, while the second was positioned at a distance of 15 cm from the receiving surface. The speed of the receiving surface was 60 cm h⁻¹, while the rate for the outlet surface was 1 cm s⁻¹. After 2 hours of spinning a nanofibrous structure of about 200 µm thick was obtained with a length of about 1.2 m and a width of 80 cm. The average nanofibre diameter changed as a function of depth from 470 nm at one side of the structure to 450 nm at the other side. The side with the largest diameters corresponds to the fibers obtained from the outlet surface positioned at 15 cm from the receiving surface, while the smallest diameters (at the other side of the nanofibrous structure) are obtained from the outlet surface positioned at 20 cm from the receiving surface.

## Claims

1. An electrospinning device for producing fibrous structures, said electrospinning device comprising :
- a set of outlets (5) for outputting solution or melt,
- a receiving surface (8) for receiving output from said set of outlets (5), wherein said receiving surface (8) is adapted to move in a first direction parallel to said receiving surface (8), said movement being responsible for the lengthwise production of said fibrous structures,
- a voltage source (1) for generating a potential difference between said set of outlets and said receiving surface,
**characterized in that** said electrospinning device is adapted for providing a predetermined distance profile for the distance between the outlets (5) and the receiving surface (8) along said first direction.

2. An electrospinning device according to claim 1, wherein the predetermined distance profile is a decreasing or increasing distance profile.

3. An electrospinning device according to claim 2, wherein said distance profile is a monotonously decreasing or monotonously increasing distance profile.

4. An electrospinning device according to any of the previous claims, wherein said set of outlets (5) comprises at least two subsets of outlets (5), wherein each of said subset consists of outlets (5) equidistant to said receiving surface (8) and wherein the distance between each subset and the receiving surface (8) is settable according to said predetermined distance profile along said first direction.

5. An electrospinning device according to any preceding claim, **characterized in that** said set of outlets is comprised in a plane inclined at an angle relatively to the receiving surface.

6. An electrospinning device according to any preceding claim, **characterized in that** at least two neighbouring outlets (5) of said set of outlets (5) are separated from one another by a distance of at least 1 cm.

7. An electrospinning device according to any preceding claim, wherein the distance between the outlets (5) within each of said set of outlets (5) is adapted for obtaining a fibrous structure comprising at least 50% of fibers substantially free of cross-links to neighboring fibers.

8. An electrospinning device according to any preceding claim, wherein said set of outlets (5) is adapted to be movable reciprocally in a direction parallel to said receiving surface (8) and perpendicular to said first direction.

9. An electrospinning device according to any preceding claim, wherein said device comprises control means (10) for varying the distance between the outlets and the receiving surface for varying the diameter of the produced fibres.

10. A method for producing fibrous structures, said method comprising the steps of:
- providing a set of outlets (5) for outputting solution or melt,
- providing a receiving surface (8) for receiving output from said set of outlets (5)
- moving said receiving surface (8) in a first direction parallel to said receiving surface (8),
- applying a potential difference between said set of outlets (5) and said receiving surface (8),
- during said moving and applying, providing a solution or melt to said outlets (5),
wherein the distance between the outlets (5) and the receiving surface is set according to a predetermined distance profile along said first direction.

11. A method according to claim 10, wherein the predetermined distance profile is a decreasing or increasing distance profile.

12. A method according to claim 11, wherein said distance profile is a monotonously decreasing or monotonously increasing distance profile.

13. A method according to any of claims 10 to 12, the method further comprising the step of moving reciprocally at least one of said set of outlets (5) and/or said receiving surface (8) in a direction parallel to said receiving surface (8) and perpendicular to said first direction.

14. An electrospun fibrous structure comprising fibres, wherein the diameter of said fibres varies according to a predetermined profile along a dimension of said electrospun fibrous structure and wherein the variance of the fibres diameter in any section perpendicular to said dimension, is below 10%.

15. An electrospun fibrous structure according to claim 14, wherein the diameter of said fibres varies according to a predetermined profile along a dimension of said electrospun fibrous structure.

16. An electrospun fibrous structure according to any of claims 14 to 15, the structure comprising at least 50% of straight fibers, wherein at least 50% of straight fibers consists of 50% or more fibres having segments substantially straight over a distance of 5 µm.

17. An electrospun fibrous structure according to any of claims 14 to16, comprising at least 50% of fibers that is substantially cross-link free with respect to neighboring fibers.

18. An electrospun fibrous structure according to any of claims 14 to 17, comprising at least 50% of randomly oriented fibers.

19. An electrospun fibrous structure according to any of claims 14 to 18 having a porosity of at least 65%.

20. An electrospun fibrous structure according to any of claims 14 to 19 wherein 50% or more of its fibers have an average diameter between 3 and 2000 nm.

21. An electrospun fibrous structure according to any of claims 14 to 20, said fibrous structure comprising two or more adjacent layers, wherein each layer having two neighboring layers is composed of fibers having an average diameter smaller than the average diameter of the fibers of one of its neighboring layer and larger than the average diameter of the fibers of its other neighboring layer.

22. A controller for controlling the provision of a predetermined distance profile for the distance between outlets (5) and a receiving surface (8) along a direction of continuous production of fibrous structure in an electrospinning device according to claims 1 to 9.
